

Sept. 20, 1927.

1,643,241

E. GATHMANN

INGOT MOLD AND INGOT

Filed Jan. 18, 1927

Fig. 1.



Fig. 2.



Fig. 3.



Emil Gathmann  
by his Attorneys  
Borden & Wright

## UNITED STATES PATENT OFFICE.

EMIL GATHMANN, OF BALTIMORE, MARYLAND.

## INGOT MOLD AND INGOT.

Application filed January 18, 1927. Serial No. 161,807.

This invention relates to the construction and contour of metallic ingot molds and to the contour of ingots cast within the mold chambers, and particularly to molds of the class in which the largest cross sectional area of the ingot is cast uppermost, the mold chamber having for the greater part of its volume, metallic heat-absorbing walls—the value or rate of which decreases from the bottom of the mold upwardly, a relatively small section at the upper portion of the mold having walls constructed of refractory material of low-heat-absorptive value.

The object of my present invention is to so shape the walls of the mold chamber that they will more effectively promote progressive solidification of degassified ingot metal from the bottom upwardly to insure soundness, and at the same time to so shape the ingot in its vertical contour that it can be more readily reduced in cross sectional area and in fewer initial mill passes than has heretofore been found practicable.

In the accompanying drawings, which are largely diagrammatic:

Figure 1 shows a vertical section through an ingot mold embodying my invention.

Figure 2 shows a vertical perspective elevation of an ingot embodying my improvements cast in a mold of the kind illustrated in Figure 1.

Figure 3 is an illustration of an initial reduction pass in a rolling mill of an ingot embodying my improvements.

As is now well-known to those familiar with the art and as described in numerous patents heretofore granted to me, sound homogeneous ingot structure is obtained most economically when an ingot is so cast that approximately 85% of its volume is formed and completely solidified in a heat-absorbing metallic mold having a big-end-up chamber, and substantially 15% of its volume is formed in a mold top or shrink head casing constructed of heat conserving material.

I have found that certain contours and definite relations of various ingot dimensions to one another are of economical and technical value in producing uniformly sound ingots for most economical reduction by the rolling action of a blooming mill or the like. In working and squaring up a steel ingot to form a bloom, (which is accomplished during the first reduction passes) it is desirable to work the cast metal and reduce the size of

the crystalline, surface dendritic structures by compressing all of the sides of the body of the ingot before elongating to any considerable degree any one part of the relatively coarsely crystalline metal originally forming the ingot. Hence, for most efficient blooming mill practice the difference in cross sectional area of the ingot from top to bottom should be as small as possible, being, however, great enough to insure of interior soundness of the ingot structure upon its solidification.

In the usual big-end-up mold, as generally used prior to my present invention, it has been the practice to form the metallic chamber walls with vertically-extending single-plane or substantially straight faces from the bottom or necked-in portion to the top of said metallic mold chamber, such walls having a uniform upward and outward taper. I have found that heretofore in order to insure uniform interior soundness throughout the body of the steel ingot structure, i. e., in the lower and body portions as well as in the upper part of the ingot, which is fed by the shrink head or reservoir of molten metal contained in the poor heat conducting portion of the mold, a degree of taper relative to the longitudinal axis of the chamber is necessary that makes difficult and costly the rolling of the ingot because of the increased number of preliminary squaring or blooming passes required. This I have remedied by applying certain different contours or degrees of taper to definite portions of the mold chamber length and the ingots formed therein. By means of this differential taper, the lower portion of the walls of the chamber can be tapered to the desired extent to insure ingot soundness and to a greater degree than has heretofore been deemed practicable, and yet the total taper of the chamber and ingot is considerably less than that heretofore considered necessary for ingot soundness. In this manner I produce not only a more uniformly sound structure but one more readily reduced to a bloom contour without danger of excessive fracture of the cast, coarsely crystallized ingot skin in the initial mill passes.

Other features of my invention are hereinafter specified more fully.

An essential characteristic of an ingot mold in its function of forming a sound,

homogeneous ingot is that it shall promote progressive solidification of the molten mass within the mold chamber from the bottom upwards in order that there may be at all 5 times a reservoir of hotter molten metal superimposed upon the earlier solidifying lower portions until solidification of the entire mass has been completed.

This method of casting ingots is described 10 and claimed in my U. S. Patent No. 1,049,573 of January 7, 1913. Since the issue of this patent, many types of molds have been proposed and patented for carrying 15 out the basic method of manufacturing steel ingots disclosed therein and many millions of tons of sound ingots have been produced in accordance with this method in both big-end-down and big-end-up types of molds.

20 When ample taper of the chamber walls is provided, the big-end-up type of mold has been found by those familiar with the art to be by far the most efficient and practical construction for carrying out the fundamental 25 requirement in the production of uniformly sound and homogeneous ingots. Mill ingots of the big-end-up type with sufficient taper to insure soundness throughout their body length, however, have heretofore been 30 more difficult and costly to roll and reduce initially into blooms than ingots having substantially parallel walls, or big-end-up and big-end-down types having but relatively slight taper.

35 Although my invention may be applied to big-end-up molds of any kind, I have shown in Figure 1 a big-end-up ingot mold M of the Gathmann type. The walls A of the mold body are constructed of heat-absorbing 40 material and the walls S of the top portion of the mold are constructed of heat-insulating material in a manner now well-known to those familiar with the art. The vertical height of the heat-absorbing walls defining 45 the mold chamber is designated at H and N, the vertical height of the heat-insulating portion by H' and the entire or total height of the chamber at Y. Lugs of any suitable construction for lifting the mold 50 during handling or stripping operation for the removal of the ingot I are shown at L and L'. S is the shrink head casing or mold top made of refractory material having poor heat-conducting qualities. E, B, C and D 55 are various sections of the mold chamber from the bottom to the top respectively. Corresponding portions of the ingot are designated at EI, BI, CI and DI. b' is the lowest horizontal cross section of the ingot 60 mold chamber and ingot, from which substantially straight outwardly tapered walls radiate upwardly to c', these walls having a greater taper per inch of vertical height than the cross sections beginning at c' and 65 tapering upwardly and outwardly to d'.

Dotted lines d in the same plane as the walls radiating from b' to c' are shown ending at d<sup>2</sup>, which would be the upper terminal of the mold cavity if the taper from the cross section b' were continued, as is the case in the one-plane old type chamber walls. The height of the chamber section E is designated by N, the height of the taper of chamber B by O, that of the chamber C by P, and the shrink head portion D by H'. The bottom of the mold is preferably closed with a sealing or closure plug V and the refractory poor-heat conducting mold top S is preferably supported on the mold by means of removable blocks as shown at T. 70 The shrink head casing has its cross sectional dimension indicated at W. The shrink head portion S' of the ingot I shown in Figure 2 is somewhat shorter than the length of the mold top or shrink head casing S due to contraction of the ingot during solidification.

In Figure 3 rolls X and X' are shown reducing the section of the ingot I, part of the ingot being broken away for convenience of illustration.

The preferred ratio of the various proportions of the mold chamber and ingot are substantially as follows:

When b' equals 17 $\frac{1}{2}$ ", H equals 4  $\times$  b', and c' should equal b' plus (O-ft.  $\times$   $\frac{1}{2}$ "), d' equals c' plus (P-ft.  $\times$   $\frac{1}{8}$ "), O equals approximately  $\frac{3}{5}$  of H, and P equals approximately  $\frac{2}{5}$  of H. From this formula, which I have compiled from experiments in determining the most efficient ingot practice, both as to solidification of the metal in the ingot and ease of rolling mill operations, I have found that the taper from b' to c' should be approximately  $\frac{1}{2}$ " per foot through the height O, and the taper from c' to d' should be approximately  $\frac{1}{8}$ " per foot through the height P. In the illustration given a straight taper from b' to d<sup>2</sup> would amount to 3", but by the use of my differential taper the total difference in the taper from b' to d' is only 2 $\frac{1}{2}$ ". As previously stated, it has heretofore been the practice to employ a continuous taper from b' to d<sup>2</sup> and such ingots, although generally sound when sufficient taper is employed, have been found more difficult to reduce in rolling practice than when my present invention of differential taper in chamber sections O and P is employed. The liquid steel in the shrink head portion S' of the ingot when amounting to approximately 12% or more of the volume of the ingot feeds downwardly so as to insure of a solid ingot interior to a depth of approximately one and one-half to two diameters of the shrink head dimension W. The shrink head dimension W should for technical reasons be approximately the dimension of b' or at any rate, not much greater than the same.

As previously stated, I have found that the hot molten metal in the shrink head feeds downwardly to and supplies hot metal to the contracting, solidifying lower ingot portion 5 somewhat beyond the horizontal dimensions  $c'$  and if  $c'$  were the actual base or bottom of the ingot, the  $\frac{1}{8}$ " taper per foot from  $c'$  to  $d'$  would be ample to insure sound interior 10 ingot structure when employing such a short ingot and relatively large shrink head chamber. The influence of the hot metal in the shrink head does not, however, usually exceed beyond one-half of the length of the mold chamber H and, therefore, I make the 15 length P somewhat less than half of the length of the chamber so as to insure of the action of the shrink head molten metal feeding to or slightly through the portion of the ingot at the cross section  $c'$ .

20 By means of the relatively increased taper of the mold walls and the ingot formed therein from section  $b'$  to  $c'$  of the chamber, I have found that the metal freezes in a uniformly sound condition from the bottom 25 of the mold upwardly and that all the shrinkage cavity or pipe and porosity due to decrease of section from liquid to solid is contained in the upper two-thirds of the shrink head S', as shown by dotted lines at F of the 30 ingot I illustrated in Figure 2.

Referring now to Figure 3, the rolls X and X' are so spaced that a single pass through the rolls will work all the metal of the ingot on the two sides being rolled and the ingot 35 being turned 90° on its longitudinal axis and given a second pass, all the metal on the surface of the ingot will be initially worked and reduced from the usual coarse crystallization of an ingot casting to a semi-forged 40 state. These initial passes must, however, not be of such a severe degree that the free sides of the ingot not being worked on during the initial passes will split and tear, due to overstress of the unforaged metal. In 45 practice it has been found that an initial reduction of 2" or at most  $2\frac{1}{2}$ " is the maximum that the cast steel in the ingot will ordinarily withstand without cracking and producing surface flaws.

50 In accordance with the old method of straight plane walls of big-end-up mold chambers and ingots, the taper which would produce interior soundness in the dimension of ingot specified amounts to 3", as previously stated, in its height H, from  $b'$  to  $d'$ . By my new improvement of differential 55 tapered walls the amount of taper in the example before given on the section of the mold chamber and ingot shown at O would 60 amount to  $\frac{1}{2}$ " per foot or a taper of  $1\frac{3}{4}$ " from  $b'$  to  $c'$  for height O. The taper from  $c'$  to  $d'$  of  $\frac{1}{8}$ " per foot would amount to  $\frac{7}{4}$ " or slightly over  $\frac{1}{4}$ " for height P. The 65 total difference in dimension at any point of the ingot would, however, amount to only

2", or, to be exact,  $2\frac{1}{4}$ ", as against a total taper of 3" as used in the old practice. It will, therefore, be readily seen that an economy in rolling the improved contour of the ingot I is obtained, as the  $2\frac{1}{4}$ " difference 70 in maximum size of ingot can be readily rolled and the skin portion suitably forged with an initial reduction of  $2\frac{1}{2}$ " in one pass of the rolls, whereas in the 3" maximum difference of cross section two passes 75 are required for the initial skin forging. The economy thus effected is considerable, inasmuch as the four sides of a rectangular ingot of my differential vertical wall contour obviously require only two passes as 80 against the four passes necessary in the old type of ingot wall contour. The points  $c'$  and length of chamber O and P may be varied somewhat for different weight ingots, but the length P should not exceed two-fifths 85 of the total ingot length, as this is the limit of feeding capacity of a shrink head casing containing from 12% to 16% of the volume of the fluid metal forming the ingot.

I claim for my invention:

1. An ingot mold comprising a heat-absorbing body portion and a heat-insulating upper part, the mold chamber in said body portion being defined by metallic heat-absorbing walls which taper upwardly and outwardly in the same general direction from bottom to top of said chamber, the taper of the lower portion of said chamber walls being considerably greater than the taper of the upper portion thereof. 90

2. An ingot mold comprising a heat-absorbing body portion and a heat-insulating upper part, the mold chamber in said body portion being defined by metallic heat-absorbing walls of a flat or plane contour which taper upwardly and outwardly in the same general direction from bottom to top of said chamber, the taper of the lower portion of the said chamber walls being considerably greater than the taper of the upper portion thereof. 95

3. In a metallic ingot mold, an ingot-forming chamber defined by metallic heat-absorbing walls of a flat or plane contour, all tapering upwardly and outwardly from bottom to top of said chamber, the taper of the lower three-fifths being considerably greater than the taper of the upper two-fifths of the height of such chamber. 100

4. In a metallic ingot mold of the big-end-up type, an ingot mold chamber characterized by metallic heat-absorbing walls which taper upwardly and outwardly in the same general direction, the upper portion of said walls having less than half the taper per inch of the lower portion of the walls. 105

5. A big-end-up ingot having a body portion with an outward and upward taper, the upper part of the ingot body which tapers in the same general direction as the lower 110

part having considerably less taper per inch of height than the lower portion of the ingot.

6. A big-end-up ingot having its base portion rounded and necked-in, and having a body portion with an outward and upward taper, the upper part having considerably less taper per inch of height than the lower portion.

10 7. A big-end-up ingot having a body portion with an outward and upward taper, the upper part having considerably less taper per inch of height than the lower por-

tion, and having also a necked-in portion at its top.

15 8. A big-end-up ingot having its base portion rounded and necked-in, and having a body portion with an outward and upward taper, the upper part of the ingot having a considerably less taper per inch of height than the lower portion, and having a necked-in portion at its top.

20 In testimony whereof, I have hereunto subscribed my name.

EMIL GATHMANN.